

## United States Patent [19]

Miller et al.

[11] 3,853,497

[45] Dec. 10, 1974

[54] LOW POUR VACUUM GAS OIL  
COMPOSITIONS[75] Inventors: **Kenneth D. Miller**, Nederland; **Levi C. Parker**, Port Arthur, both of Tex.[73] Assignee: **Texaco, Inc.**, New York, N.Y.[22] Filed: **Nov. 8, 1972**[21] Appl. No.: **304,676**[52] U.S. Cl. .... **44/62, 44/70, 44/80,**  
137/13[51] Int. Cl. .... **C10I 1/14**[58] Field of Search .... **44/62, 70, 80; 137/13**

## [56] References Cited

## UNITED STATES PATENTS

|           |         |                |          |
|-----------|---------|----------------|----------|
| 2,020,714 | 11/1935 | Wulff et al.   | 252/56 R |
| 2,091,627 | 8/1937  | Bruson         | 252/56 R |
| 2,891,991 | 6/1959  | Stewart et al. | 44/70 X  |
| 2,917,375 | 12/1959 | Hudson         | 44/80 X  |
| 2,967,816 | 1/1961  | Hudson         | 44/62 X  |

## FOREIGN PATENTS OR APPLICATIONS

1,398,539 6/1964 France ..... 44/62

Primary Examiner—Patrick P. Garvin

Assistant Examiner—Andrew H. Metz

Attorney, Agent, or Firm—T. H. Whaley; C. G. Ries

[57]

## ABSTRACT

A vacuum gas oil fuel composition suitable for pipeline transportation of substantially reduced pour point comprising a wax containing vacuum gas oil base stock having incorporated therein a minor amount of high asphaltene residuum such as an Arabian Light 1,050,°F. + residuum and a pour depressing amount of an interpolymeric poly(n-alkylacrylate) of a molecular weight between about 3,000 and 100,000 wherein said alkyl is of at least 18 carbons and at least 70 wt. % of said alkyl is between about 20 and 24 carbons inclusively, the  $C_{20}$  to  $C_{24}$  alkyl group consisting of between about 2 and 65 wt. % of  $C_{20}$  alkyl, between about 18 and 65 wt. %  $C_{22}$  alkyl and between about 8 and 35 wt. %  $C_{24}$  alkyl.

2 Claims, No Drawings

## LOW POUR VACUUM GAS OIL COMPOSITIONS

## APPLICATION OF RELATED INTEREST

Coassigned, copending application Ser. No. 266,839, filed June 27, 1972.

## BACKGROUND OF INVENTION

This invention relates to improved vacuum gas oil compositions of significantly reduced pour point and to transportation of these compositions in pipelines. More particularly, it pertains to vacuum gas oil compositions comprising a wax containing vacuum gas oil base stock having a pour depressing amount of an interpolymeric poly(n-alkylacrylate) and a minor amount of high asphaltene residuum incorporated therein.

Gas oils are generally defined in the petroleum industry as hydrocarbon fractions in a crude oil ranging between the kerosene fraction and the lubricating oil fraction. However, the boundaries of the gas oil fraction can overlap into adjacent fractions within the standard definition employed. The vacuum gas oils are normally the heavier, that is, higher boiling portions of the gas oil fraction being recovered as its name denotes under vacuum, e.g., 0.05-0.2 atmosphere.

Petroleum hydrocarbon oils employed in cold climates or exposed to low temperature frequently require the use of an additive to maintain their fluidity, e.g., in pipeline transportation, or to meet pour point specifications. Additives that are effective for this are called pour depressors. The art discloses numerous classes of pour depressors.

Pour depressant additives are mostly high molecular weight organic compositions prepared by alkylation of benzene, naphthalene or derivatives thereof, by polymerization of low molecular weight methacrylates, and by the condensation polymerization of various types of these compounds. Many of these additives are not entirely suitable in vacuum gas oils because of their high cost, high concentration required or because they are relatively ineffective in reducing the pour point of vacuum gas oil base stocks containing higher molecular weight waxes.

Although a wide variety of different pour depressants mentioned above are useful for incorporating in heating oils, diesel fuels and many other liquid hydrocarbon oils, they have been found, in general, to be relatively ineffective in decreasing the pour point of vacuum gas oil base stocks containing the higher molecular weight waxes. The poor performance of these additives may result from the structural and/or molecular weight difference of waxes occurring in the various oil fractions.

In the past, two means which have been employed in attempting to improve the pour point characteristics of wax containing vacuum gas oils are the solvent extraction (dewaxing) process and the centrifugal dewaxing method. Solvent dewaxing involves introducing and recovering a large amount of valuable solvent material which necessarily results in an expensive operation. In the centrifugal method of separating the wax it is necessary to first add a cutter stock such as naphtha and then cool the gas oil mixture to a low temperature such as about -25°F. which is time consuming and also a costly processing step. Still another approach called for the thermocracking of the waxy vacuum gas oil base stocks. However, the thermocracking process, although resulting in the reduction of the pour point of

10°-20°F. leads to the loss of a substantial volume of vacuum gas oil. There is, therefore, a need in the art for an economic means of reducing pour point of the high pour (e.g. 60°-100°F.) wax containing gas oil stocks.

5 In the aforementioned coassigned, copending application, Ser. No. 266,839, filed June 27, 1972, a major step was taken in fulfilling this need in that a particular interpolymeric poly(n-alkylacrylate) is described which is effective in reducing the pour point of vacuum 10 gas oils at a reasonable cost. However, there is a continuing search to improve the effectiveness of this found interpolymeric poly(n-alkylacrylate) pour depressor.

A main object of the present invention is to improve 15 the pour point characteristics of wax containing vacuum gas oils without utilizing elaborate and expensive solvent extraction or centrifugal dewaxing procedures.

Another object of this invention is to provide improved 20 vacuum gas oil compositions prepared by incorporating therein a pour depressing amount of an oil soluble interpolymeric poly(n-alkylacrylate) and a vacuum residuum of high asphaltene content in a wax containing vacuum gas oil.

Still another object of the invention is to improve the 25 wax containing vacuum gas oil base stocks so they may be handled, e.g., in pipeline transportation with greater ease and flexibility in climates where ambient temperatures are near their pour points.

## SUMMARY OF INVENTION

We have discovered and this constitutes our invention 30 a vacuum gas oil fuel composition of reduced pour point comprising a vacuum gas oil having a wax content of between about 0.5 and 20 wt. % and containing the pour reducing combination of between about 1 and 20 wt. % of a high asphaltene containing petroleum residuum and between about 0.002 and 3 wt. % of a pour 35 depressing quantity of an oil soluble poly(n-alkylacrylate) of a molecular weight between about 3,000 and 100,000 wherein said alkyl is of at least 18 carbons and at least 70 wt. % of said alkyl is about 20 to 24 carbons, the C<sub>20</sub> to C<sub>24</sub> n-alkyl group consisting of between about 2 and 65 wt. % C<sub>20</sub> alkyl, between 40 about 18 and 65 wt. % C<sub>22</sub> alkyl and between about 8 and 35 wt. % C<sub>24</sub> alkyl.

In another aspect, this invention relates to a process 45 for the pipeline transportation of the above mentioned fuel oil compositions.

Surprisingly, it has been found that the addition of a minor amount of a high asphaltene residuum together 50 with a small amount of an oil soluble poly(n-alkylacrylate) to a vacuum gas oil or mixture of gas oils as defined yield a fuel oil composition of much lower pour point than when either residuum or polyacrylate alone is added to the vacuum gas oil base stock. An unexpected synergistic action is achieved through the addition of the residuum together with the polyalkylacrylate interpolymer.

60 The waxy type vacuum gas oil base stocks contemplated herein have a wax content between about 0.5 and 20 wt. %, a pour point between about 60° and 100°F., an atmospheric boiling point between about 450° and 1,050°F., an API gravity between about 20 and 35 and are normally derived from the distillation of crude oils such as Arabian Light crude oils at vacuum pressures ranging between about 0.05 to 0.2 atm-

spheres. Typical vacuum gas oils which may be employed are Desulfurized Arabian Light Vacuum Gas Oil (DS Arabian Lt. VGO), Desulfurized Lago Medio Vacuum Gas Oil (DS Lago Medio VGO), Arabian Light Vacuum Gas Oil (Arabian Lt. VGO), Lago Medio Vacuum Gas Oil (Lago Medio VGO) and Amna Vacuum gas oil, etc. whose physical properties are set out in Table I as follows:

As heretofore stated, the pour point depressant additives useful in the practice of this invention are the gas oil soluble interpolymeric poly(n-alkylacrylate)s of a molecular weight between about 3,000 and 100,000, preferably between 4000 and 52,000, most preferably between 15,000 and 35,000 wherein said alkyl is of at least 18 carbons, at least 70 wt. % of said alkyl is between 20 and 24 carbons inclusively, the C<sub>20</sub> to C<sub>24</sub>

TABLE I

| GAS OIL                      | Amna Vac.<br>Gas Oil | D.S. Lt.<br>Arab. VGO | D.S. Lago<br>Medio VGO | Lago Medio<br>VGO | Arab. Lt.<br>VGO |
|------------------------------|----------------------|-----------------------|------------------------|-------------------|------------------|
| Boiling Range, °F.           | 650-900              | 650-1050              | 650-1050               | 450-1050          | 650-1050         |
| Pour Point, °F. (ASTM D-97)  | +95                  | +90                   | +90                    | +90               | +95              |
| Sulfur, wt. %                | 0.30                 | 0.23                  | 0.16                   | 1.4               | 2.6              |
| Wax Content, wt. %           | 17.3                 | ~11                   | ~10                    | ~10               | ~11              |
| Kin. Visc. at 122°F., cs.    | 11.5                 | 37.2                  | 27.0                   | —                 | —                |
| Kin. Visc. at 130°F., cs.    | —                    | —                     | —                      | 16.2              | 58.0             |
| API Gravity, 60°F.           | 32.6                 | 25.5                  | 28.1                   | 27.0              | 20.0             |
| Gas Oil Distillation, Vol. % |                      |                       |                        |                   |                  |
| Recovered at °F              |                      |                       |                        |                   |                  |
| IBP* - 5 Vol. %              | 587°F.               | —                     | —                      | 453-538°F.        | 681-749°F.       |
| 10-20                        | 636-698              | —                     | —                      | 586-642           | 773-804          |
| 30-40                        | 708-734              | —                     | —                      | 689-743           | 825-848          |
| 50                           | 750                  | —                     | —                      | 778               | 868+             |
| 60-70                        | 771-796              | —                     | —                      | 810-855           | —                |
| 80-90                        | 823-858              | —                     | —                      | 882+              | —                |
| 95 - EP*                     | 876-899              | —                     | —                      | —                 | —                |

\*IBP - Initial Boiling Point

\*\*EP - End Point

The high asphaltene residuum component suitable for use in the fuel oil compositions of this invention include a wide variety of residual fuel oil bottoms such as Arabian Light (650°F. + or greater) residuum, Lago Medio (650°F. + or greater), a thermally cracked heavy fraction of Amna Crude (650°F. + or greater), West Texas Sour Residuum (650°F. + or greater) and thermal cycle fuel oil from various crude sources. Preferably, the residuous stocks employed will have an asphaltene content of about 4 to about 15 wt. % and a carbon residue of about 5 to 25 wt. %. Gravity of the residuous stocks will range from about 5° to about 20° API (60°F.). Although the amount of residuum in the fuel oil compositions of this invention can be varied over a wide range, the maximum amount which can be utilized is about 20 wt. % and preferably will be from about 1 to 15 wt. % based on the weight of the composition. It is to be noted this residuum component not only synergistically enhances the pour depressing effect of the poly(n-alkylacrylate) pour depressor but also functions as a fuel that is an energy supplying ingredient. Suitable properties of typical residuous fractions which may be utilized in the novel compositions of this invention are set forth in Table 2 below:

30 alkyl group consisting of between about 2 and 65 wt. % of C<sub>20</sub> alkyl, between about 18 and 65 wt. % C<sub>22</sub> alkyl, and between about 8 and 35 wt. % C<sub>24</sub> alkyl. The interpolymers are derived from standard polymerization techniques such as polymerizing the alkylacrylate monomers in the presence of acrylate polymerization catalyst, e.g., azo catalyst such as azobisisobutronitrile described in U.S. Pat. No. 2,471,959 or the well known peroxide catalysts such as benzoyl peroxide and lauroyl peroxide, utilizing catalyst quantities of between about 0.1 and 5 wt. %. Polymerization is normally conducted at a temperature between about 50° and 150°C., preferably at 80°-100°C., utilizing a nitrogen blanket to prevent oxidation of the catalyst. During polymerization normally a periodic sample is taken for refractive index (RI) determination. The polymerization reaction is continued until the refractive index remains steady. The reaction time is normally between about 1 and 10 hours.

35 The n-alkylacrylate monomers from which the interpolymeric poly(n-alkylacrylate) products are prepared are made by standard esterification techniques through the reaction of acrylic acid with n-alkanol mixtures wherein the reactive n-alkanols in said mixture have at

TABLE 2

| Tests on Residue Stocks           |                           |                                 |                            |                                |                                 |
|-----------------------------------|---------------------------|---------------------------------|----------------------------|--------------------------------|---------------------------------|
|                                   | Thermal Cycle<br>Fuel Oil | 1050°F.<br>Lago Medio<br>Resid. | 900°F. +<br>Amna<br>Resid. | 1050°F. +<br>Arab<br>Lt.Resid. | Cracked<br>950°F.<br>Amna Crude |
| Pour Point, °F.                   | +35                       | 120+                            | 120+                       | 120+                           | +70                             |
| Sulfur, wt. %                     | 0.87                      | 2.8                             | 0.31                       | 3.2                            | 0.29                            |
| Vis. Kin., at 122°F. cs.          | 392                       | —                               | —                          | —                              | —                               |
| Vis. Kin., at 210°F. cs.          | 46.2                      | 1700                            | 23.9 at 300°F.             | 469                            | —                               |
| API Gravity, at 60°F.             | 8.0                       | 9.8                             | 14.8                       | 9.2                            | —                               |
| Carbon Residue, wt. %             | —                         | 20.4                            | 17.5                       | 17.1                           | —                               |
| Asphaltene basis N-C <sub>5</sub> | —                         | 12                              | 9                          | 9                              | —                               |
| Insoluble, wt. %                  |                           |                                 |                            |                                |                                 |

least 18 carbons and 70 wt. % thereof are in the n-alkanol group of 20 to 24 carbon atoms, said group consisting of between about 2 and 65 wt. % of eicosanol, between about 18 and 65 wt. % of docosanol and between 8 and 35 wt. % tetracosanol. One suitable source of alcohol mixtures are the alcohols sold under the tradename "Alfol" by Continental Oil Co. "Alfol" are impure mixtures of n-alkanols of various chain lengths, the remainder consisting of hydrocarbons, ketones and hindered unreactive alcohols. Typical analysis of two suitable examples of the "Alfol" alcohols are as follows:

| Typical Properties                              | Alfol 20+R | Alfol 22+R |
|-------------------------------------------------|------------|------------|
| Approx. homolog Distribution 100% alcohol bases |            |            |
| $C_{18}$                                        | 2          | 1          |
| $C_{20}$                                        | 60         | 5          |
| $C_{22}$                                        | 20         | 60         |
| $C_{24}$                                        | 10         | 21         |
| $C_{26}$                                        | 5          | 9          |
| $C_{28}^{(+)}$                                  | 3          | 4          |
| Alcohol Content, approx. Wt. %                  | 70         | 60         |
| Hydroxyl No.                                    | 123        | 90         |
| Hydroxyl No., 100% alcohol basis                | 176        | 150        |
| Sap. No.                                        | 3          | 6          |
| $I_2$ No.                                       | 12         | 13         |
| Carbonyl, % (C=O)                               | 0.2        | 0.3        |
| Melting Point range, °F.                        | 113-135    | 113-136    |
| Color, Gardner                                  | 12         | 18         |

A standard means of acrylate monomer precursor preparation is reacting (esterifying) the alcohol mixture with acrylic acid in the presence of an esterification catalyst such as p-toluenesulfonic acid and a polymerization inhibitor, e.g., hydroquinone desirably in the presence of an azeotroping agent for water by-product removal such as benzene. The esterification is conducted, for example, at a temperature between about 190° and 200°F. and is continued until the amount of water by-product is removed as overhead indicating that the esterification is essentially complete.

The novel fuel compositions of this invention can be prepared in a variety of ways. For example, the residuum component can be mixed with the base vacuum gas oil or gas oils and the polyacrylate can be admixed as a solution in toluene, xylene, light lube oil or in the vacuum gas oil itself. One preferred solvent to facilitate introduction of the polyacrylate pour depressor into the vacuum gas oil base stock is a solvent such as a light lubricating oil of a kinematic viscosity of between about 2 and 4 cs. at 100°F. to form between about 10 and 50 wt. % polyacrylate lube oil concentrate.

Generally, the residuum and gas oil components are heated to a temperature of about 175° to 300°F., preferably at 175° to 250°F. prior to the addition of the polyacrylate following which addition the resulting mixture is heated at a temperature of about 175° to 300°F., preferably 175° to 250°F., for about 0.2 to 1.5 hours or more to insure complete solution of the inter-polymeric blend. It is important that the polyacrylate pour depressor be introduced at a temperature above the solution point of the wax component. If the polyacrylate is mixed with a vacuum gas oil at a temperature substantially below the solution point of a substantial portion of the wax component, there is little or no pour depressing effect afforded by the polyacrylate-residuum combination.

In another aspect, this invention relates to improved process for the transportation of the novel fuel oil compositions described in detail above.

The improved process of this invention for the pipeline transportation of viscous fuel oils comprises introducing into the pipeline a fuel oil composition comprising a major amount of vacuum gas oil boiling between 450° and 1,050°F. and a minor amount (i.e. not over 20 percent by weight and preferably about 1 to about 15 wt. % based on the weight of the composition) of a high asphaltene residuum and an effective pour depressant amount of a poly(n-alkylacrylate) as heretofore described.

The following examples further illustrate the invention but are not to be construed as limitations thereof.

### EXAMPLE I

This example describes two species of the poly(n-alkylacrylate), Polyacrylate A and B, contemplated herein and their method of preparation.

Polyacrylates A and B are described and prepared as follows:

#### Monomer Synthesis

The alcohols employed to prepare the A and B monomers were as follows:

| Typical Properties                                     | Alcohol A | Alcohol B |
|--------------------------------------------------------|-----------|-----------|
| Approx. Homolog Distribution 100% alcohol basis, wt. % |           |           |
| $C_{18}$                                               | 5         | 0         |
| $C_{20}$                                               | 39        | 12        |
| $C_{22}$                                               | 27        | 47        |
| $C_{24}$                                               | 14        | 21        |
| $C_{26}$                                               | 7         | 10        |
| $C_{28}$                                               | 3         | 5         |
| $C_{30}^{(+)}$                                         | 5         | 5         |
| $C_{32}^{(+)}$                                         | —         | —         |
| Alcohol Content, approx.                               | 70        | 60        |
| Hydroxyl No.                                           | 123       | 90        |
| Sap. No.                                               | 3         | 6         |
| $I_2$ No.                                              | 12        | 13        |
| Carbonyl, % (as C=O)                                   | 0.2       | 0.3       |
| Melting Range, °F.                                     | 113-135   | 113-136   |
| Color, Gardner                                         | 12        | 18        |

From Alcohols A and B there were respectively derived Mono-Acrylate A and B as follows:

| Material               | Wt. (g.) | Moles |
|------------------------|----------|-------|
| Hydroquinone           | 2        | 0.02  |
| p-Toluenesulfonic acid | 5.6      | 0.036 |
| Alcohol A              | 952      | 2     |
| Alcohol B              | 1245     | 2     |
| Acrylic acid, glacial  | 144      | 2     |
| Benzene                | 536      | —     |

All the above charge except the acrylic acid was put together under nitrogen at about 60°C. (140°F.). The acrylic acid was then added with stirring and the mixture brought to reflux, with a pot temperature of about 90°C. (194°F.). Nitrogen was introduced below the surface of the liquid reaction mixture at a rate of between about 40 and 45 mls./minute as the water of reaction was azeotroped off at a reflux rate of 4 mls./minute. About 96 percent of the theoretical amount of water was removed in 12 hours and all the water was removed in 21 hours. Benzene was removed by stripping the product to 15 mm Hg pressure at a pot temperature of

about 60°C. (140°F.). Physical data for the monomer product was as follows:

| Physical Data for Monomer | Mono-Acrylate A | Mono-Acrylate B |
|---------------------------|-----------------|-----------------|
| Sap. No.                  | 115             | 95              |
| Neut. No.                 | 1.3             | 1.1             |
| Hydroxyl No.              | 8               | 14              |
| Sp. Grav., 150°F./60°F.   | 0.8316          | 0.8310          |
| Refractive Index          | 1.4450          | 1.4465          |
| Kin. Visc., cs.           |                 |                 |
| 150°F.                    | 7.39            | 8.84            |
| 210°F.                    | 3.9             | 4.50            |
| Dialysis Residue, %       | < 3             | < 3             |
| Melting Point, °C.        | 36              | 38              |

### Polymer Synthesis

The monomer produced above was subjected to polymerization to form the poly(n-alkylacrylate) pour depressant product. The procedure employed was as follows:

In the procedure 200 grams of Mono-Acrylates A and B were heated in separate runs to 85°C. (185°F.) over a 20 minute period under prepurified nitrogen introduced into the reaction system at a rate of 120 mls./minute. The nitrogen flow was then reduced to 40 mls./minute and 4 grams of azobisisobutronitrile were added. The reaction mixture was stirred and readings of the refractive index of the mixture were taken at 1/2 hour intervals, and the reaction was continued until the refractive index is constant, that is,  $\pm 3$  units in the fourth decimal place. The total reaction time required was about 1.5 hours.

The product was cooled and analyzed and the resultant polyacrylates gave the following analysis:

| Physical Data           | Polyacrylate a | Polyacrylate B |
|-------------------------|----------------|----------------|
| RI                      | 1.4545         | 1.4540         |
| Sp. Grav., 150°F./60°F. | 0.8580         | 0.8495         |
| Melting Point, °C.      | 47             | 48             |
| Kin. Visc., cs 150°F.   | 196            | 115            |
| 210°F.                  | 81             | 49             |
| Dialysis, % Residue     | 55             | 48             |
| Mo. Wt. Residue         | 23,000         | 20,000         |

### EXAMPLE II

This example illustrates the composition of the invention, the outstanding pour depressing effect of the polyacrylate and the residuum and their synergistic interaction to reduce pour.

TABLE 4

### Enhancing Effectiveness of PAA Pour Depressant in Gas Oil Stock by Addition of Vacuum Residuum

| BLEND                         | A    | B    | C    | D    | E    | F    | G    | H    |
|-------------------------------|------|------|------|------|------|------|------|------|
| Arabian Lt. DS HVGO, wt. %    | 100  | 100  | 90.0 | 90.0 | 95.0 | 95.0 | 97.5 | 97.5 |
| Arabian Lt. Vac. Resid. wt. % | 0    | 0    | 10.0 | 10.0 | 5.0  | 5.0  | 2.5  | 2.5  |
| PAA, wt. %                    | None | 0.10 | None | 0.10 | None | 0.10 | None | 0.10 |
| <u>Test Results</u>           |      |      |      |      |      |      |      |      |
| *Pour Point, °F.              |      |      |      |      |      |      |      |      |
| ASTM Upper Maximum            | +80  | +65  | +75  | +50  | +70  | —    | +80  | +50  |
| Kin. Visc., cs at 210°F.      | +80  | +60  | +75  | +45  | +75  | +55  | +75  | +50  |
|                               | 5.69 | 5.61 | 7.47 | 7.35 | 6.42 | 6.39 | 6.00 | 5.99 |

\*Maximum pour point provides an indication of the stable pour point of a fuel oil. In the maximum determination, the gas test oil is heated to 220°F. for about 30 minutes, following which it is cooled rapidly to 0°F. by placing in a cold box. This low temperature nucleates the wax present. After 12 or more hours, the fuel oil is removed and allowed to warm at ambient temperature. An ASTM pour point is then obtained. Residual fuel oil blends containing distillate stocks sometimes exhibit pour reversion tendencies (pour increases) upon storage. The above blends containing PAA + residuum showed no pour reversion characteristics.

A series of blends was prepared utilizing desulfurized heavy vacuum gas oil as the base stock and Arabian Light 1,050°F. plus residuum by mixing the two components at 200°F. for 30 minutes. The polyacrylate component employed was Polyacrylate A described in Example I. Polyacrylate A (PAA) was introduced into the base stock and residuum mixture at 200°F. The outstanding reductions in pour points as well as the synergistic action achieved through the Polyacrylate-residuum combination can be seen in the following tables.

Following Table 3 describes the vacuum gas oil base stock and the vacuum residuum employed and Table 4 sets forth pour depressing data. Blends D, F and H are representative of the compositions of the invention and Blends A, C, E and G are comparative blends. As can be seen by subsequent Table 4, when only vacuum residuum is employed as the pour depressing ingredient even in amount of 10 wt. %, essentially no pour depression takes place. When the polyacrylate is employed as the sole pour depressor at 0.1 wt. % amount the pour depression is about 15°F. However, when the combination of residuum and polyacrylate is employed the average pour depression is about 30°F. Fuel oils of the type presented in Table 4 normally carry an ASTM pour requirement of +60°F. maximum. As can be seen, addition of the residuum alone produces essentially no pour reduction in the vacuum gas oil. Addition of the pour depressor alone brought the pour to +60°-65°F., which is borderline to failing. The synergistic effect of adding residuum and pour depressor to the vacuum gas oil reduced the pour point to about 50°F., well within pour point specification.

TABLE 3

| Test Results on Component Stocks |                                            |                           |
|----------------------------------|--------------------------------------------|---------------------------|
| Stock                            | Arabian Lt. Desulfurized Hvy. Vac. Gas Oil | Arabian Lt. Vac. Residuum |
| Gravity, °API                    | 28.2                                       | —                         |
| Sp. Grav., at 60/60°F.           | —                                          | 1.013                     |
| Kin. Visc., cs. at 100°F. (SUS)  | 37.73 (176)                                | —                         |
| 150°F.                           | 13.35                                      | —                         |
| 210°F.                           | 5.69                                       | 660.8                     |
| Pour, ASTM Upper, °F.            | +80                                        | +95                       |
| Sulfur, wt. % (X-Ray)            | 0.20                                       | 3.9                       |
| Carbon Residue, Wt. %            | —                                          | 19.4                      |

We claim:

1. A vacuum gas oil fuel oil composition comprising a major amount of vacuum gas oil boiling between about 450° and 1,050°F. and having a wax content between about 0.5 and 20 wt. % containing 1). between about 1 and 20 wt. % of an asphaltene petroleum residuum having an asphaltene content of between about 4 and 15 wt. % and an API Gravity of between about 5° and 20° and a carbon residue of between about 5 and 25 wt. % and 2). between about 0.002 and 3 wt. % of an interpolymeric poly(n-alkylacrylate) of a molecular weight between about 3,000 and 100,000 wherein said n-alkyl is at least 18 carbons and where at least 70 wt. % of said n-alkyl is of 20 to 24 carbons consisting of between about 2 and 65 wt. %  $C_{20}$  alkyl, between about 18 and 65 wt. %  $C_{22}$  alkyl, and between about 8 and 35 wt. %  $C_{24}$  alkyl, said poly(n-alkylacrylate) incorporated in said base stock at a temperature above the solution point of said wax.

2. In the pipeline transportation of viscous fuel oil the improvement which comprises introducing into the

said pipeline a fuel composition comprising a major amount of vacuum gas oil boiling between about 450° and 1,050°F. and having a wax content between about 0.5 and 20 wt. % containing 1). between about 1 and 20 wt. % of an asphaltene petroleum residuum having an asphaltene content of between about 4 and 15 wt. % and an API Gravity of between about 5° and 20° and a carbon residue of between about 5 and 25 wt. % and 2). between about 0.002 and 3 wt. % of an interpolymeric poly(n-alkylacrylate) of a molecular weight between about 3,000 and 100,000 and wherein said n-alkyl is at least 18 carbons and where at least 70 wt. % of said n-alkyl is of 20 to 24 carbons consisting of between about 2 and 65 wt. %  $C_{20}$  alkyl, between about 18 and 65 wt. %  $C_{22}$  alkyl, and between about 8 and 35 wt. %  $C_{24}$  alkyl, said poly(n-alkylacrylate) incorporated in said base stock at a temperature above the solution point of said wax.

20

\* \* \* \* \*

25

30

35

40

45

50

55

60

65